

J. F. EBERT.

PROTECTOR.

APPLICATION FILED APR. 18, 1916.

1,295,714.

Patented Feb. 25, 1919.

Fig. 1.



Fig. 2.



Joseph F. Ebert Inventor:

# UNITED STATES PATENT OFFICE.

JOSEPH FRANCIS EBERT, OF NEW YORK, N. Y.

## PROTECTOR.

1,295,714.

Specification of Letters Patent.

Patented Feb. 25, 1919.

Application filed April 18, 1916. Serial No. 91,926.

*To all whom it may concern:*

Be it known that I, JOSEPH FRANCIS EBERT, a citizen of the United States, residing at New York, in the county of New York and State of New York, have invented certain new and useful Improvements in Protectors, of which the following is a full, clear, concise, and exact description.

This invention relates to devices designed 10 to protect electric circuits and apparatus from abnormal currents, such as high potential electricity or lightning.

In protectors it is common practice to have a pair of opposing electrodes maintained electrically separate by means of a dielectric which is usually a sheet of mica. In protectors having a small air-gap the use of mica is objectionable, if not impossible, because of the difficulty from a commercial 20 standpoint to hold a very thin sheet thereof to a uniform thickness. Due to the characteristics of mica, the loss resulting from working it into perfect dielectrics is very high. This waste factor adds considerable 25 to the cost of mica dielectrics. It is the object of this invention to provide a comparatively cheap dielectric material equally as efficient as mica.

The dielectric contemplated by this invention comprises a piece of insulating material or composition made of constituents having a mineral origin and held together by a suitable binding agent. These constituents may consist of powdered or granular mica and talc held together by a suitable cement. The composition formed by these ingredients may have one of the side portions cut away approximately to the center, which affords passage for the discharge 35 of electricity thereacross through air.

In the accompanying drawings, Figure 1 is a perspective of a protector embodying the features of this invention; and Fig. 2 is a side elevation of the dielectric of the 45 invention.

Interposed between a pair of electrodes 1-1, such as carbon blocks, is a dielectric 2. One side of the dielectric 2 is cut away preferably as shown at 3. The cut-away portion of the dielectric allows the passage 50 of the discharge of electricity thereacross through the air, and when the electrodes 1-1 are of carbon, also permits the disintegrated particles of the carbon usually 55 caused by such a discharge, to fall from be-

tween the electrodes 1-1 when the protector shown in Fig. 1 is placed in a horizontal position. The dielectric 2 may comprise a piece of insulating material made of powdered or granular mica and talc held together by a suitable binding agent such as shellac, etc. In case mica and talc mixed with shellac are used for the dielectric, these materials may be mixed dry in any convenient manner and then formed into sheets 60 in accordance with any approved method, such as being passed repeatedly between heated rolls and finally delivered upon a cooling table. These sheets may then be sized to any dimensions corresponding to 65 those of the dielectrics used in standard forms of protectors. The protector shown in Fig. 1 may be held in place in a circuit in any well-known manner.

From the above it is obvious that a dielectric embodying the features of this invention may consist of an insulating material made entirely of either granular mica or talc, or said material may comprise a composition made of both of these substances having a greater or less percentage of either. While the preferred embodiment of this invention has been herein particularly shown and described, many modifications may readily be made without departing 70 from the spirit of this invention.

What is claimed is:

1. In a high potential electricity protector, suitable electrodes opposing each other, and a thin dielectric of uniform thickness interposed between said electrodes, said dielectric comprising a composition consisting of mica and talc reduced to a very fine state of subdivision and bound together by a suitable binding agent. 95

2. In a high potential electricity protector, suitable electrodes opposing each other, and a thin dielectric of uniform thickness interposed between said electrodes, said dielectric comprising a piece of insulating material made of constituents reduced to a very fine state of subdivision and having a mineral origin, said particles being held together by a suitable binding agent. 100

3. In a high potential electricity protector, suitable electrodes opposing each other, and a thin dielectric of uniform thickness interposed between said electrodes, said dielectric comprising a piece of insulating material made of constituents reduced to a very 105

fine state of subdivision and held together by a suitable binding agent, one of said constituents being mica.

4. In a high potential electricity protector, 5 suitable electrodes opposing each other, and a thin dielectric of uniform thickness interposed between said electrodes, said dielectric comprising a piece of insulating material made of constituents reduced to a very fine 10 state of subdivision, said material being substantially non-heat softenable.

5. In a high potential electricity protector, suitable electrodes opposing each other, and a thin dielectric of uniform thickness interposed between said electrodes, said dielectric comprising a piece of insulating material made of mineral constituents reduced to a 15 very fine state of subdivision and held to-

gether by a suitable binding agent, said insulating material having a side portion 20 thereof cut away approximately to the center.

6. In a high potential electricity protector, suitable electrodes opposing each other, and a thin dielectric of uniform thickness interposed between said electrodes, said dielectric comprising a piece of insulating material made of mineral constituents reduced to a very fine state of subdivision and held together by a suitable binding agent, said insulating material having provision for permitting the discharge of electricity thereacross through air.

In witness whereof, I hereunto subscribe my name this 15th day of April, A. D. 1916. 35

JOSEPH FRANCIS EBERT.